

## UNITED STATES PATENT OFFICE.

ROSCOE C. MENERAY, OF COUNCIL BLUFFS, IOWA.

## RADIATOR-SEALING COMPOSITION.

No Drawing.

Application filed May 18, 1927. Serial No. 192,486.

This invention relates to a composition of matter found to be effective in mending leaky radiators of engines, water jackets, engine blocks, boilers, or other containers of water heated either to the boiling point or to approximately 180 degrees F.

One of the objects of the invention is to provide a composition consisting of few ingredients which may be conveniently obtained without undue expense, which may be deposited in the form of a powder, in the heated water of the radiator or other container when found to be leaky.

Another object is to provide a composition for the purposes described, which will form a solid body at the place or places of leakage more quickly than ordinary.

Still another object is to provide a composition of matter which, when used for these purposes will remove all adhesions from the injured metallic parts at the places of leakage before the mending occurs.

Still another object is to provide such ingredients for the composition that large as well as small abrasions, cracks, seams or perforations may be mended.

The invention includes a specifically prepared or rectified flour derived from flaxseed.

The composition consists of ingredients, in weight, approximately as follows:

|                            | Pounds.          |
|----------------------------|------------------|
| Pulverized aluminum (fine) | 62 $\frac{1}{3}$ |
| Granulated aluminum        | 1 $\frac{1}{3}$  |
| Sodium bicarbonate         | 21 $\frac{1}{3}$ |
| 35 Sodium carbonate        | 4                |
| Rectified flaxseed flour   | 66 $\frac{2}{3}$ |

In preparing this composition of matter the granulated and finely pulverized aluminum are thoroughly mixed with the rectified flaxseed flour, and thereafter the remaining ingredients are added, and mixed therewith.

For mending leaks in a radiator of average size, approximately three ounces are used. By operation of the engine the water in the radiator may attain a heat of 180 degrees or more.

The composition is then placed in the radiator, about ten minutes being required for the aluminum to crystallize in the perforations, cracks or other openings.

For mending large cracks in a radiator or engine-block about four to six ounces of the composition are required.

The rectified flour is prepared as follows:

After the flaxseed has been ground or crushed, it is treated in a manner to remove the bran and all residue, the parts remaining after treatment being flour, each particle of which carries a certain proportion of oil.

In operation the composition is moved by a movement of the hot water to the leak, and in passing through the perforation, seam or crack, the soda causes removal of any adhesions or accumulation of foreign substances at these places, and the aluminum and flour unite and solidify and form metallic bodies or plugs in the openings to effectively prevent leakage.

The proportions for the ingredients mentioned are those found to be the best. However these proportions may be changed somewhat if desired, and I do not wish to limit myself in this respect.

The advantage in the use of both granulated and finely pulverized aluminum is that leaks may be mended more quickly than would result if the finely pulverized aluminum only was employed.

I claim as my invention,—

1. A radiator sealing composition comprising finely pulverized aluminum, granulated aluminum, sodium carbonate, sodium bicarbonate and rectified flaxseed flour, each particle of said flaxseed flour containing oil.

2. A radiator sealing composition comprising aluminum, sodium carbonate, sodium bicarbonate, and flaxseed flour having the bran removed therefrom but retaining the natural oil in each particle thereof.

In testimony whereof, I have affixed my signature.

ROSCOE C. MENERAY.